

Aug. 24, 1943.

H. T. SMYTH

2,327,674

METHOD OF HEAT CASTING REFRACTORY BLOCKS

Filed May 22, 1940

*Fig. 1.*



*Fig. 3.*



*Fig. 4.*



*Fig. 5.*



*Fig. 6.*



Inventor  
HAROLD T. SMYTH

By *Dreyer Cole & Garner*

Attorneys

## UNITED STATES PATENT OFFICE

2,327,674

## METHOD OF HEAT CASTING REFRactory BLOCKS

Harold T. Smyth, Louisville, Ky., assignor to Corhart Refractories Company, Louisville, Ky., a corporation of Delaware

Application May 22, 1940, Serial No. 336,645

4 Claims. (Cl. 49—79)

Useful refractories can be made by electrically melting refractory compositions and casting to shape in suitable molds. During the subsequent cooling, liquid resolidifies to a nonporous highly crystalline refractory, the crystallization proceeding gradually inward from each mold surface in proportion to the latent heat dissipated from the surface. Since, however, the volume of any crystalline refractory material is less than the volume occupied when melted, a pipe will be produced if the mold is just filled. This internal flow in a casting is obviously objectionable for any refractory which is required to resist failure by corrosion, as, for example, glass refractories. One method of decreasing the pipe is to supply additional molten material from a font reservoir above the gate from which additional material can drain into the casting after partial solidification has occurred. This technique is limited by the fact that the font casting is also freezing at substantially the same rate as the main casting, so that in order for molten material to be available at the last stages of crystallization of the main casting, the font must be substantially as large as the casting itself. This is obviously uneconomical, and in practice a font with perhaps 10% of the volume of the casting is normally employed which although relatively efficient still leaves a pipe.

This economical procedure was further improved by the Fulcher Patent 1,700,288 and during the past few years thousands of tons of heat cast refractories have been made in that way. In that procedure a sand mold surrounded by insulating powder is filled with molten material through a font mold of insufficient volume to prevent pipe formation. In both the font mold and the sand mold solidification takes place from the outside, draining of perhaps 30 to 50% of the molten material in the font occurring, however, due to the solidification in the sand mold with attendant decrease in volume. When the font shell is exhausted of its molten core however, further decrease in volume produces a pipe within the casting. When solidification of the casting is almost complete, the font mold and insulating powder are removed from the top of the casting and the font shell broken away exposing the pipe. A new font mold is placed around the opening and the pipe filled with additional molten material.

While, as stated, this procedure has been followed in the production of a large quantity of refractories it has been attended with considerable loss due to cracked castings. Hitherto an

erroneous belief as to the determining factors in this cracking has prevented the reduction of loss, but I have discovered the correct theory and have invented a procedure by which it may be reduced if not entirely prevented and such invention forms the subject-matter of this application. Briefly stated it involves the early removal of the font shell after the initial pouring, and the proper thermal protection of the upper face of the cast block immediately adjacent to the pipe during the period of solidification of such initial pour. It also includes smoothing such face of the block immediately after removing the font shell.

Fig. 1 is a cross section through the sand mold and iron font mold.

Fig. 2 is a view similar to Figure 1, showing the font mold removed and the top of the sand mold and font shell covered with insulating powder.

Fig. 3 is a cross section, showing the font shell and top sand slab removed.

Fig. 4 is a cross section showing the application of the heat-insulating cover and the covering of the casting with the insulating powder.

Fig. 5 is a view similar to Figure 4, illustrating the casting approaching solidification and the formation of septa.

Fig. 6 is a cross section somewhat similar to Fig. 4, illustrating the use of a plaque to prevent the insulating powder from entering the pipe in the casting.

Referring to the accompanying drawing which represents successive operations in carrying out my improved procedure, Figure 1 illustrates a condition existing at such time after the initial pour that a rigid wall *m* has formed inside the sand mold *l* and the iron font mold *2* due to the loss of heat from these surfaces and the molten material has just started to drain downward from the font shell *n* through the gate *4* in the top slab *1a* of the sand mold *l*. At this stage the iron font mold *2* is removed, and the font shell and top of the sand mold covered with insulating powder *5* (see Figure 2) which delays the freezing of molten material in the font shell so that a larger proportion drains into the casting. In Figure 2, the refractory in the sand mold has partly solidified and the molten material has drained completely from the font leaving in the latter the successive septa *6a* extending across the pipe in the font shell. The pipe *6* in the block is just starting to form immediately below the gate. At this time (which is definite for a definite size) the font shell is pulled off and the top sand slab *1a* removed (see Figure 3). I have discovered that if the font shell is removed at this stage the

irregular refractory protuberances left by such removal around the rim of the gate can be easily removed by a scraper, together with any sand adhering to the top of the casting, while after a longer period of waiting the refractory protuberances are strong and the sand immediately beneath the font shell tends to fuse tightly to the casting. The upper end of the pipe is then covered by a refractory and heat insulating cover 11, and the top of the casting re-covered with the insulating powder 5 (see Figure 4). When solidification of the casting is almost complete, a pipe 6 will be formed crossed irregularly with septa 6<sup>b</sup> (see Figure 5). At this stage the insulating powder is brushed off the top of the casting around the pipe and the cover 11 removed, the font mold put back into place over the pipe, the septa broken through with a bar and the pipe refilled with molten refractory. This refilling process can be repeated if found necessary. The casting is finally annealed.

Particularly with thin blocks breakage is apt to occur if excessive force is required to break through the font septa 6<sup>a</sup>. I have discovered, however, that these septa are easily broken down if this is done shortly after formation. It is therefore advantageous to break these down one by one as they are formed which can be done by removing momentarily the refractory gate cover 11 at intervals and poking with a bar. In this way the pipe can be kept open to its maximum width and the pieces which fall into the liquid 9 are frozen into the bottom portion of the casting one by one rather than all at once in a small area, where they may produce strains or inhomogeneities in crystal growth.

The refractory cover for the gate is conveniently made of a good grade of fire brick which may be backed, if greater insulation is desired, with a less refractory insulating brick, or a composite refractory-insulating brick may be used.

To prevent the insulating powder applied to the top of the casting from being knocked into the pipe during the removal and replacing of the cover, which may occur several times during a casting operation, I have found it convenient to make the cover in two sections. The first section consists of a plaque, 11<sup>a</sup> Figure 6, as thick as the desired layer of insulating powder 5, with a hole in the center as large as the gate 4 in 50 the top slab. This section of the cover is left in position throughout the casting operations and serves primarily as a retaining wall to exclude from the pipe and the casting any of the insulating powder. The second section of the 55 cover is the part 11, which covers the hole in the first named plaque and can be easily removed and replaced without disturbing the insulating powder.

Having thus described my invention what I 60 claim as new and desired to secure by United States Letters Patent is:

1. The method of making solid cast refractories which includes pouring molten material into a mold provided with a gate through a font mold of volume insufficient to prevent pipe formation, 5 removing the font mold, breaking away the font shell formed therein at the completion of the draining of molten material therefrom, protecting the space which was below the gate with a heat conserving cover during a substantial part of the solidification which produces the pipe, thereafter removing the cover and filling the pipe with additional molten material.

2. The method of making solid cast refractories which includes pouring molten material into 15 a mold provided with a gate through a font mold of volume insufficient to prevent pipe formation, removing the font mold, breaking away the font shell formed therein at the completion of the draining of molten material therefrom, smoothing the top of the casting around the space which was below the gate, protecting such space with a heat conserving cover during a substantial part of the solidification which produces the pipe, thereafter removing the cover and filling the pipe with additional molten material.

3. The method of making solid cast refractories which includes pouring molten material into a mold provided with a gate through a font mold of volume insufficient to prevent pipe formation, 30 removing the font mold, breaking away the font shell formed therein at the completion of the draining of molten material therefrom, protecting the space which was below the gate with a heat conserving cover during a substantial part of the solidification which produces the pipe, 35 removing said cover from time to time and punching down the septa as formed in the pipe during such solidification, thereafter removing the cover and filling the pipe with additional molten material.

4. The method of making solid cast refractories which includes pouring molten material into a mold provided with a gate through a font mold of volume insufficient to prevent pipe formation, 45 removing the font mold, breaking away the font shell formed therein at the completion of the draining of molten material therefrom, protecting the gate by a heat conserving cover during a substantial part of the solidification which produces the pipe, removing the cover, refilling the pipe with additional molten material through a font mold of volume insufficient to prevent pipe formation and thereafter removing the font mold, breaking away the font shell formed therein at the completion of the draining of molten material therefrom, protecting the space which was below the gate by a heat conserving cover during a substantial part of the solidification of the added material, thereafter removing the cover and refilling with molten material the pipe produced during such solidification.

HAROLD T. SMYTH.